

# United States Patent

Nihyakumen et al.

[15] 3,653,903

[45] Apr. 4, 1972

## [54] DIAZO-TYPE MULTICOLOR REPRODUCTION PROCESS

- [72] Inventors: Kouzi Nihyakumen, Hirakata; Taizo Yokoyama, Osaka; Yasuo Ueda, Kobe; Yasutoki Kamezawa; Tatsuo Aizawa, both of Osaka, all of Japan
- [73] Assignee: Mita Industrial Company, Ltd., Osaka, Japan
- [22] Filed: July 31, 1970
- [21] Appl. No.: 59,923

### [30] Foreign Application Priority Data

- Aug. 2, 1969 Japan..... 44/60756
- [52] U.S. Cl..... 96/49, 96/91, 117/36.8,  
117/36.9, 250/65 T
- [51] Int. Cl..... G03c 5/18
- [58] Field of Search ..... 96/49.75, 91; 117/36.7, 36.8,  
117/36.9; 250/65 T

### [56] References Cited

#### UNITED STATES PATENTS

- 2,541,178 2/1951 Slifkin..... 96/91 X  
2,789,904 4/1957 Benbrook et al..... 96/91 X  
3,224,878 12/1965 Klimkowski et al. .... 96/49  
3,454,764 7/1969 Collier et al. .... 96/49

## FOREIGN PATENTS OR APPLICATIONS

1,000,151 8/1965 Great Britain..... 96/49

## OTHER PUBLICATIONS

Landau, R. et al., J. of Photo. Sci., Vol. 13, 5/1965, p. 444-451

Dinaburg, M. S., "Photosensitive Diazo Cpd.", 1964, The Focal Press, p. 50-54.

Van der Grinter, The Photographic Journal, 1952, Vol. 92B, p. 43-48.

Primary Examiner—Charles L. Bowers, Jr.  
Attorney—Sherman and Shalloway

### [57] ABSTRACT

A process for the diazo-type multicolor reproduction which comprises (A) exposing to light a diazo-type photosensitive material having a photosensitive layer containing at least one diazonium salt (c) and a coupler (b) having a substantially lower rate of coupling with the diazonium salt (c) than that of resorcin, said coupler being present in the photosensitive material in an amount of not greater than 1 mole per mole of said diazonium salt (c), and (B) heating a layer of at least one thermovolatile or thermosublimative coupler (a) disposed in a face-to-face contact with said photosensitive material at a predetermined portion, said steps being carried out coincidentally or in the order of (A) to (B) or (B) to (A), and then developing the exposed photosensitive material. photosensitive material.

5 Claims, 3 Drawing Figures

ORIGINAL

1 2 3  
ORIGINAL



Patented April 4, 1972

3,653,903

2 Sheets-Sheet 1

ORIGINAL

Fig. 1



Fig. 2



PREPARATION OF ORIGINAL FOR  
MULTICOLOR DEVELOPMENT



DEVELOPMENT



Patented April 4, 1972

3,653,903

2 Sheets-Sheet 2

Fig. 3



## DIAZO-TYPE MULTICOLOR REPRODUCTION PROCESS

This invention relates to a process for the diazo-type multicolor reproduction and photosensitive materials in use for said process. More specifically, it relates to a process for the diazo-type multicolor reproduction by which portions of a photosensitive paper corresponding to predetermined portions of the original can be colored selectively to different hues without substantial mingling of colors, and to photosensitive materials in use for said process.

We previously proposed a process for the diazo-type multicolor reproduction based on the discovery that predetermined portions of an original can be reproduced into different hues regardless of difference or similarity of the light transmission in the original by conducting the steps of (A) exposing to light a diazo-type photosensitive material containing at least one diazonium salt (c) and (B) heating a layer of at least one thermovolatile or thermosublimative coupler (a) disposed in a face-to-face contact with a predetermined portion of said diazo-type photosensitive material, said steps being carried out coincidentally or in an order of (A) to (B) or (B) to (A), and then developing the exposed photosensitive material in the presence of a coupler (b) having a lower coupling rate under developing conditions than said thermovolatile or thermosublimative coupler (a).

In case the above process is conducted by employing a commercially available, diazo-type, two-component photosensitive material, at portions corresponding to predetermined portions of an original there can be formed an azo dyestuff having a different hue from that of a dyestuff formed at other portions, but it has been found that at said portions corresponding to the predetermined portions of the original there is also formed the dyestuff of the same kind as that formed at other portions and mingling of colors is caused to occur, which renders the color contrast indistinct. We have traced the origin of this undesirable phenomenon and found that since conventional diazo-type, two-component photosensitive materials contain a great excess of a coupler, for instance, in an amount of 4 moles per mole of the diazonium salt, this coupler (b) couples with the diazonium salt in competition with the thermovolatile or thermosublimative coupler (a), which results in undesired mingling of colors.

We furthered our research and now found that in the above-mentioned diazo-type multicolor reproduction process predetermined portions of the resulting copy can be colored selectively in different hues from other portions without substantial mingling of colors by choosing as coupler (b) a coupler having a substantially lower rate of coupling with a diazonium salt (c) of the photosensitive layer than that of resorcin and making said coupler present in the photosensitive layer in an amount of not greater than 1 mole per mole of the diazonium salt.

Thus, in accordance with this invention, there is provided a process for the diazo-type multicolor reproduction which comprises conducting the steps of (A) exposing to light a diazo-type photosensitive material having a photosensitive layer containing at least one diazonium salt (c) and a coupler (b) having a substantially lower rate of coupling with the diazonium salt (c) than that of resorcinol, said coupler (b) being present in the photosensitive material in an amount of not greater than 1 mole per mole of said diazonium salt (c), and (B) heating a layer of at least one thermovolatile or thermosublimative coupler (a) disposed in a face-to-face contact with said photosensitive material at a predetermined portion, said steps being carried out coincidentally or in an order of (A) to (B) or (B) to (A), and then developing the exposed photosensitive material.

Any coupler that has a substantially lower rate of coupling with a diazonium salt (c) contained in a photosensitive material than that of resorcinol, preferably that of 2,3-dihydroxyphthalene, can be used as coupler (b) in the process of this invention. Typical examples of such coupler (b) are as follows:

Phenol Derivatives  
2,5,6-Trimethylphenol

|    |                                                                |
|----|----------------------------------------------------------------|
|    | 2-Hydroxymethylphenol                                          |
|    | $\beta$ -(2-Hydroxyphenyl)-propionic acid                      |
|    | 2-( $\omega$ -Phenylaminomethyl)-phenol                        |
|    | $\beta$ -(4-Methyl-2-hydroxyphenyl)-glutaric acid              |
| 5  | 2,5-Dimethyl-6-(N-dimethylaminomethyl)-phenol                  |
|    | 1,3-Dimethyl ether of pyrogallol                               |
|    | $\alpha$ -Resorcylic acid ethanolamine                         |
|    | $\beta$ -Resorcylic acid                                       |
| 10 | N-Lauryl-p-aminophenol                                         |
|    | N-Acyl-m-aminophenol                                           |
|    | Meta-hydroxy-acetoanilide                                      |
|    | Ortho-N-hydroxyphenyl-monoguanidine                            |
|    | Para-N-hydroxyphenyl-biguanidine                               |
| 15 | 2,5-Dimethyl-4-morpholinomethyl phenol                         |
|    | 2-Methyl-5-isopropyl-morpholinomethyl phenol                   |
|    | 4-Morpholinomethylresorcinol monomethyl ether                  |
|    | 3,3',5-Trihydroxydiphenyl                                      |
|    | 3,3',5,5'-Tetrahydroxydiphenyl                                 |
| 20 | 2,2',4,4'-Tetrahydroxydiphenyl                                 |
|    | 2,4,4'-Trihydroxydiphenyl-2'-sulfonic acid                     |
|    | 2,4,6,3',5'-Pentahydroxydiphenyl                               |
|    | 2,2',4,4'-Tetrahydroxydiphenyl sulfide                         |
|    | 3-(Aminophenylsulfonylamine) phenol                            |
| 25 | 1,3-Dihydroxy-5-chlorobenzene                                  |
|    | 4-Bromoresorcinol                                              |
|    | 4-Iodoresorcinol                                               |
|    | 4-Fluororesorcinol                                             |
|    | N- $\beta$ -Hydroxyethyl-2-resorcylamide                       |
|    | $\alpha$ -Resorcylamide                                        |
| 30 | N-Phenyl- $\alpha$ -resorcylamide                              |
|    | 1,3-Dihydroxybenzene-5-sulfonic acid                           |
|    | 3,5-Dihydroxytoluene                                           |
|    | 1,3,5-Resorcylic acid ethanolamine                             |
|    | 1,2,5-Resorcylic acid ethanolamine                             |
| 35 | 1,3,5-Resorcylic acid anilide                                  |
|    | 1,3,5-Resorcylic acid amide                                    |
|    | 4-Chloro-3,5-dihydroxybenzoic acid amide                       |
|    | 3,5-Dihydroxybenzoic acid amide                                |
|    | <i>m,m'</i> -Trimethylenedioxy diphenyl                        |
|    | <i>m,m'</i> -1-Methyltrimethylenedioxy diphenyl                |
|    | 6,6'-Dimethyl-3,3'-trimethylenedioxy diphenyl                  |
|    | <i>m,m'</i> -( <i>p</i> -Phenylene-dimethylenedioxy)-diphenyl  |
|    | 6,6'-Dihexyl-3,3'-isopropylidenedioxy diphenyl                 |
|    | Resorcinol acetaldehyde                                        |
|    | Resorcinol-phosgen reaction product                            |
| 40 | Bis-(2,4-diphenylsulfide)                                      |
|    | Bis-(2,4-diphenylsulfoxide)                                    |
|    | Phloroglucinol                                                 |
|    | 1,3,5-Trihydroxy-2-methylbenzene                               |
|    | Fluoroglucinol monoethyl ether                                 |
|    | 3,3',5'-Trihydroxydiphenyl                                     |
|    | 2,4,4'-Trihydroxydiphenyl                                      |
|    | 3,3',5,5'-Tetrahydroxydiphenyl                                 |
|    | 4,4',6,6'-Tetrahydroxydiphenyl                                 |
| 45 | Phloroglycide                                                  |
|    | Naphthols                                                      |
|    | 2,3-Dihydroxynaphthalene-6-sulfonic acid                       |
|    | 2-Naphthol-3,6-disulfonic acid                                 |
|    | 2,7-Dihydroxynaphthalene-3-sulfonic acid                       |
|    | 2,8-Dihydroxynaphthalene-6-sulfonic acid                       |
|    | 1,8-Dihydroxynaphthalene-8-sulfonic acid                       |
|    | 1-8-Aminonaphthol-5-sulfonic acid                              |
| 50 | 2,7-Dihydroxy-3,6-disulfonic acid                              |
|    | 1,8-Benzoylaminonaphthol-2-sulfonic acid                       |
|    | 1,8-Dihydroxynaphthalene-6-sulfonic acid                       |
|    | 2-Hydroxy-3-naphthionic-N- $\beta$ -hydroxyethyl amide         |
|    | $\beta$ -Hydroxynaphthionic acid aminoethylamine               |
|    | 2-Hydroxy-3-naphthionic-N,N-bis- $\beta$ -hydroxyl ether amide |
|    | 8-Hydroxy-2-naphthionic-hydroxyethyl amide                     |
| 55 | 1-(N-Carboethoxymethylamino)-8-naphthol-4-sulfonic acid        |
|    | 5-(Para-nitro)-benzamido-1-naphthol                            |
|    | 1-Hydroxynaphthyl-7-phenyl-guanidine                           |
| 60 | 2-Hydroxynaphthyl-8-biguanidine                                |
| 65 |                                                                |
| 70 |                                                                |
| 75 |                                                                |

1-Naphthol-3-(N-β-hydroxyethyl)-sulfonic amide  
 1-Naphthol-3-(N-o-methoxyphenyl)-sulfonic amide  
 Bis-[5-hydroxy-7-sulfo-naphthyl(2)]-amine  
 N,N-Bis[1-hydroxy-3-sulfo-naphthyl(6)]-thiourea  
 2,3-Dihydroxynaphthalene  
 2,7-Dihydroxynaphthalene  
 2,8-Dihydroxynaphthalene-3,6-disulfonic acid  
 2,7-Dihydroxy-1-naphthalene-methanesulfonic acid  
 1,5-Dihydroxynaphthalene  
 1,6-Dihydroxynaphthalene-3-sulfonic acid  
 1,8-Dihydroxynaphthalene-3-sulfonic acid  
 1-Hydroxy-8-aminonaphthalene-6-sulfonic acid  
 1,8-Diaminonaphthalene-4-sulfonic acid  
 2,7-Dihydroxynaphthalene-6-sulfonic acid  
 Active Methylene Group-containing Compounds  
 Acetoacetic acid cyclohexylamide  
 Acetoacetic acid benzylamide  
 Cyanoacetoanilide  
 Cyanoacetomorpholine  
 2,4-Diacetoacetoaminotoluene  
 Diacetoacetyl piperidine  
 Heterocyclic Compounds  
 1-(3'-Sulfoamide)-phenyl-3-methylpyrazolone-5  
 1-(4'-Carboxy-ethylphenyl)-3-dodecyl-pyrazolone-5  
 8-Hydroxy-1,2-naphthylimidazole  
 2-Methyl-4-hydroxybenzimidazole  
 7-Methyl-4-hydroxybenzothiazole  
 1,7-Dimethyl-4-hydroxy-benzotriazole  
 3-Hydroxythiophene-5-carboxylic acid  
 1-3-4-Cyclopentatrione  
 Compounds Expressed by the Following General Formula



wherein X stands for =O, =S or =N-Z<sub>3</sub>; Z<sub>2</sub> stands for Z<sub>1</sub> or a group



Z<sub>4</sub> stands for  
 an arylene group; Z<sub>1</sub> and Z<sub>5</sub> each are selected from hydroxyaryl groups; and Z<sub>3</sub> stands for hydrogen, or an alkyl group or an hydroxyalkyl or hydroxyaryl group which may have another substituent than the hydroxyl group.  
 N,N',N''-Tris[1-hydroxy-3-sulfonaphthyl(6)]guanidine  
 N-[1-Hydroxy-8-naphthyl]-N,N'-bis[1-hydroxy-naphthyl(6)]guanidine  
 N-2-Hydroxyethyl-N',N''-bis-[1-hydroxy-3-sulfo-naphthyl(6)]guanidine  
 N,N'-Bis[1-hydroxy-3-sulfonaphthyl(6)]guanidine  
 N,N'-Bis[1-hydroxy-8-sulfonaphthyl(6)]urea  
 N,N'-Bis[1-hydroxyphenyl(3)]thiourea  
 N,N',N''-Tris[1-hydroxyphenyl(3)]guanidine  
 4,4'-Bis{N',N''-[1-hydroxyphenyl(3)]quanidine}diphenyl  
 4,4'-Bis{N',N''-[1-hydroxy-3-sulfonaphthyl(6)]quanidine}diphenyl  
 Compounds Expressed by the Following General Formula



wherein A and A' stand for an aromatic ring which may have optional substituents other than the hydroxyl and primary amino groups.  
 Bis-[5-hydroxy-7-sulfonaphthyl(2)]-amine  
 Bis-[8-hydroxy-2,4-disulfonaphthyl(1)]-amine  
 Bis-[8-hydroxy-6-sulfonaphthyl(2)]-amine  
 Bis-[8-hydroxy-4-sulfonaphthyl(1)]-amine

## Diazocompounds Capable of Forming Bis-azo Compounds



in which X is an alkyl, alkoxy or acyl group.



in which R is -CH<sub>2</sub>OH, -C<sub>2</sub>H<sub>4</sub>OH or -C<sub>3</sub>H<sub>6</sub>OH, and n is 1-8.



in which X is a diazo group, Y is -N(R)<sub>2</sub>, R is an alkyl group, and A is a single bond, or -O-, -S- or -NHCOOC-<sub>H</sub>CONH-.



30 in which X is -O-, or -S- and R and R' stand for H-alkoxy.



65 In this invention any of the above-cited compounds listed on pages 4-9 may be used as coupler (b), but it is preferable to employ couplers having two or more hydroxyl or active methylene groups and being capable of forming polyazo dyes 70 such as bis-azo dyes and tris-azo dyes, especially couplers having two or more aromatic rings containing a hydroxyl group.

In case a coupler capable of forming a bis-azo or poly-azo dye is used, it is desired to make the coupler present in the photosensitive material in an amount of 0.5 - 0.1 mole per 75 mole of the diazonium salt (c).

In case a coupler capable of forming a bis-azo or poly-azo dye is used in combination with a coupler forming a mono-azo dye, the coupler for a bis-azo or poly-azo dye is used in an amount of 0.5 - 0.1 mole per mole of the diazonium salt and the coupler for a mono-azo dye is used in an amount of 0.9 - 0.1 mole per mole of the diazonium salt, with the proviso that the total amount of both couplers is within the range of 0.9 - 0.1 mole per mole of the diazonium salt.

Any of conventional photo-resoluble diazonium salts used as diazo-type photosensitive materials may be used as diazonium salt (c) in this invention, so far as it is capable of coupling with the above-mentioned coupler (b) under ordinary developing conditions. Examples of such diazonium salt are as follows:

- Para-phenylene-diamine-N,N-substituted compounds of the following general formula:



wherein X stands for an anion, R' and R'' each are aliphatic groups, and Z and Y denote groups which can be introduced into the benzene nucleus.

Specific examples of the compounds of this type are as follows:

- 4-Diazo-N,N-dimethyl aniline  
(referred to simply as "MA salt")
- 4-Diazo-N,N-diethyl aniline  
(referred to simply as "EA salt")
- 4-Diazo-N-ethyl-N-β-hydroxyethyl aniline  
(referred to simply as "EH salt")
- 4-Diazo-N,N-bis-β-hydroxyethyl aniline
- 4-Diazo-N-methyl-N-β-hydroxyethyl aniline
- 4-Diazo-N-ethyl-N-β-hydroxypropyl aniline
- Other diazonium salts of *p*-phenylene diamines N,N-substituted with alkyl or hydroxy-alkyl groups
- 4-Diazo-N-ethyl-N-(β-diethylamino)-ethyl aniline
- 4-Diazo-2-chloro-N,N-diethyl aniline
- 4-Diazo-2-methyl-N,N-diethyl aniline
- 4-Diazo-2-iodo-N,N-diethyl aniline
- 4-Diazo-2-trifluoromethyl-N,N-diethyl aniline
- 4-Diazo-N-ethyl-N-benzyl aniline
- 4-Diazo-N-methyl-N-benzyl aniline  
(referred to simply as "methyl benzyl")

○ Aminohydroquinone ether-type compounds of the following general formula:



wherein R, R' and R'' are alkyl or aryl groups and X stands for an anion.

Specific examples of the compounds of the above type are as follows:

- 4-Diazo-2,5-dibutoxy-N,N-diethyl aniline
- 4-Diazo-2,5-diethoxy-N-benzoyl aniline  
(referred to simply as "BB salt")
- 4-Diazo-2,5-diethoxy-N-ethyl-N-benzoyl aniline
- 4-Diazo-2,5-dibenzoyloxy-N-benzoyl aniline
- 4-Diazo-2-chloro-5-methoxy-N-benzoyl aniline
- 4-Diazo-2,5-diethoxy-N-benzoyl-methyl aniline
- 4-Diazo-2,5-diethoxy-N-benzoyloxy-methyl aniline
- Other 4-diazo-2,5-dioxyalkyl (or dioxyaryl)-N-alkyl (or aryl) compounds and derivatives thereof
- Aminodiphenyl compounds, aminodiphenyl amine compounds and their analogues of the following general formulas:



and



5

wherein X is an anion, R is a divalent aryl group, R' is a monovalent or divalent aryl or alkyl group, A is a divalent group or a direct bond and examples of the R-A-R' are diarylamine (A; -NH-), diphenyl (A; direct bond), diphenyl oxide (A; -O-), diaryl methane (A; -CH<sub>2</sub>-), stilbene (A; -CH = CH-) and diaryl or dialkyl sulfide (A; -S-).

Specific examples of the compounds of the above type are as follows:

- Para-diazophenyl amine
- 4-Diazo-2,5,4'-triethoxydiphenyl amine
- 4-Diazo-2,5,4'-triethoxydiphenyl
- 4,4'-Bis-diazo-2,2',5,5'-tetrahydroxydiphenyl methane
- Bis-diazo-8,8'-dichloro-5,5'-dimethoxy benzidine
- 4-Diazo-2,5-dimethoxyphenylethyl sulfide
- 4-Diazo-2,5-diethoxy-4'-methyl-diphenyl sulfide

○ Heterocyclic amine derivatives of the following general formula:



wherein X stands for an anion, Y and Z are groups which can be introduced into the benzene nucleus, and A is a direct bond or a divalent group such as -O-, -S- and methylene.

Specific examples of the compounds of this type are as follows:

- 4-Diazo-2,5-dibutoxy-N-phenyl morpholine
- 4-Diazo-2,5-diethoxy-N-phenyl morpholine
- 4-Diazo-2-methoxy-N-thio morpholine
- 4-Diazo-N-phenyl piperidine
- 4-Diazo-N-phenyl pyrrolidine
- 4-Diazo-2,5-di-n-butoxy-N-phenyl piperidine

Other derivatives of 4-Diazo-N-phenyl heterocyclic amines.

○ N,N-Substituted ortho-phenylene diamine derivatives and orthoamino-phenol derivatives.

Specific examples of the compounds of this type are as follows:

- 2-Diazo-4-methylmercapto-N,N'-dimethyl aniline
- 2-Diazo-5-benzoylamino-N,N'-dimethyl aniline
- 2-Diazo-1-naphthol-5-sulfonic acid

The above-mentioned diazonium compounds may be used in the form of a relatively stable salt with sulfuric acid or hydrochloric acid. They may be also used in the form of a double salt with zinc chloride, tin chloride, aluminum sulfate or the like. Further, they may be used in the state stabilized by an aryl sulfonate (in the form of a diazonium salt of an aromatic sulfonic acid), a diazosulfonate or the like. These diazonium salts may be used either singly or in the form of a mixture of 60 two or more of them.

In accordance with this invention, the above-mentioned coupler (b) is used in an amount of not greater than 1 mole per mole of such diazonium salt (c). In case the amount of the coupler (b) is more than 1 mole per mole of the diazonium salt (c), when the coupling reaction is allowed to advance between the diazonium salt (c) and the coupler (a) heat-transferred on the photosensitive layer, the coupling reaction between the diazonium salt (c) and the coupler (b) is also allowed to advance to some extent, which sometimes results in occurrence 65 of undesired mingling of colors. However, if the amount of the coupler (c) in the photosensitive layer is made less than 1 mole per mole of the diazonium salt, it is possible to form a dyestuff composed of the coupler (a) and the diazonium salt (c) selectively at portions of the photosensitive layer corresponding to predetermined portions of the original. In this

invention it is generally preferable to employ the coupler (b) in an amount of 0.2 - 0.9 mole per mole of the diazonium salt (c).

In this invention, sensitizing compositions formed from the diazonium salt (c) and coupler (b) together with optional assistants selected depending on the developing method are coated on a substrate such as paper, plastic film, textile fabric, non-woven fabric and metal foil, and thus there are formed photosensitive materials. The preparation of such photosensitive material will now be described by referring to only some examples.

## A.

## Sensitizing composition for dry development:

|                            |                                             |
|----------------------------|---------------------------------------------|
| Diazo compound (c)         | 0.2-5.0 %                                   |
| Azo coupling component (b) | 0.2-0.9 mole per mole of diazo compound (c) |
| Organic acid               | 0.1-5.0 %                                   |
| Coloring matter            | 0.001-0.025 %                               |
| Development promoter       | 1.0-10.0 %                                  |
| Extender                   | 0-2.5 %                                     |
| Solvent                    | balance                                     |

The sensitizing composition of the above recipe is coated on a substrate such as paper and plastic film, and dried to form a photosensitive sheet.

## B.

## Two-component-type sensitizing composition for wet development:

|                            |                                             |
|----------------------------|---------------------------------------------|
| Diazo compound (c)         | 0.2-5.0 %                                   |
| Azo coupling component (b) | 0.2-0.9 mole per mole of diazo compound (c) |
| Organic acid               | 0.1-5.0 %                                   |
| Extender                   | 0-2.5 %                                     |
| Stabilizer                 | 0-5.0 %                                     |
| Coloring matter            | 0.001-0.025 %                               |
| Solvent                    | balance                                     |

The sensitizing composition of the above recipe is coated on a substrate such as paper and plastic film, and dried to form a photosensitive sheet.

As the organic acid in the sensitizing composition there may be used citric acid, tartaric acid, oxalic acid, sulfamic acid, etc. As the extender there may be used dextrin, gum arabic, colloidal silica, etc. As the stabilizers there may be used 1,3,6-naphthalene, sodium trisulfonate and other aryl sulfonic acids. Polyhydric alcohols such as glycerin and ethylene glycol are used as development promoter. Coloring matters are used for indicating the photosensitive face and increasing the whiteness of the back ground, and blue dyestuffs such as methylene blue and Patent Blue are used for this purpose. As the solvent there may be used water and organic solvent such as alcohols, acetone, toluene, xylene and esters.

The multicolor reproduction using the diazo-type photosensitive materials of this invention is performed by conducting the steps of (A) exposing to light a photosensitive material containing at least one diazonium salt (c) and a coupler (b) in the above-mentioned amount and (B) heating a layer of at least one thermovolatile or thermosublimative coupler (a) disposed in a face-to-face contact with said photosensitive material at a predetermined portion, said steps being carried out coincidentally or in an order of (A) to (B) or (B) to (A), and then subjecting the exposed photosensitive material under developing conditions.

It is essential that among thermovolatile or thermosublimative coupler (a), coupler (b) and diazonium salt (c) to be used in this invention there should be established the following relations:

I. Thermovolatile or thermosublimative coupler (a) has a higher coupling rate under developing conditions than coupler (b).

II. Dyestuff (b)-(c), dyestuff (a)-(c), dyestuff (a')-(c).....formed at the development have hues different to one another.

Any coupler that can be volatilized or sublimated under heating conditions may be used as thermovolatile or thermosublimative coupler (a) in this invention. As such coupler (a) there may be mentioned phenol derivatives, hydroxynaphthalene derivatives, aniline derivatives and active methylene group-containing compounds. In view of facilitation of the heat transfer operation it is preferred that these derivatives do not contain soluble groups such as a sulfonic acid group.

Examples of these derivatives usable as coupler (a) are as follows:

## Phenol Derivatives

## Phenol

## Pyrocatechol

## Resorcinol

## Phloroglucinol

*o*-Hydroxybenzalcohol

## Resorcinol monoglycol ether

## Resorcinol diglycol ether

## Hydrotoluquinone

## Pyrogallol-4-carboxylic acid

## Vanillin

## Isovanilllic acid

## Vanilllic acid

## 5-Hydroxy-isophthalic acid

## 2-Hydroxy-terephthalic acid

2-Hydroxy-*p*-toluyllic acid3-Hydroxy-*p*-toluyllic acid5-Hydroxy-*o*-toluyllic acid6-Hydroxy-*m*-toluyllic acid5-Hydroxy-*l*-naphthionic acid

## Para-hydroxyphenylacetic acid

## 2,7-Dihydroxynaphthalene

## 2,3-Dihydroxynaphthalene

## 8-Amino-2-naphthol

## 2,2'-dihydroxy-1,1'-binaphthyl

## 4,4'-dihydroxy-1,1'-binaphthyl

## 3-carboxy-2-naphthol

## Aniline Derivatives

## Meta-aminobenzoic acid

2-Amino-*p*-cresol

## Ortho-aminophenol

## Para-aminophenol

## Para-chloroaniline

## 3,4-Diaminotoluene

## Active Methylene Group-containing Compounds

## 1-Phenyl-3-methylpyrazolone (5)

## 1-Phenyl-3-carboxypyrazolone

## Acetoacetic acid anilide

Acetoacetic-*o*-chloroanilide

## Para-hydroxybenzaldehyde

## Ortho-hydroxybenzoic acid

## Ortho-hydroxybenzyl alcohol

## 4,4-Dihydroxybiphenol

## 3,5-Dichloro-salicylic acid

## 5-Chloro-2-nitrophenol

## 2,5-Dihydroxyacetophenone

## 2,5-Dinitrophenol

## 2,4-Dinitrophenol

## 2,4-Dinitroresorcin

## 4,6-Dibromo-2-nitrophenol

## 2,5-Dimethyl hydroquinone

## Hydroxynaphthalene Derivatives

## 2,3-Dihydroxynaphthalene

 $\beta$ -Naphthol $\alpha$ -Naphthol

## 1,6-Dihydroxynaphthalene

## 2,6-Dihydroxynaphthalene

## 2,7-Dihydroxynaphthalene

In case a plurality of thermovolatile or thermosublimative couplers (a) are used, the coupling rate of the coupler (b) should be lower than that of any of couplers (a). Selection of couplers (a) and (b) meeting the above requirement may be

easily performed by those skilled in the art based on a simple experiment.

In conducting the reproduction process of this invention, at first an original for multicolor development is formed by applying at least one transparent or semi-transparent layer of a thermovolatile or thermosublimative coupler (a) onto the back surface of one or more predetermined portions of a transparent or semi-transparent original to be copied.

The so formed original for multicolor development is overlapped on a diazo-type photosensitive material containing at least one diazonium salt (c) and a coupler (b) in a manner such that the layer of coupler (a) will confront the photosensitive surface of the photosensitive material, and the light-exposure and heating are effected coincidentally with the above overlapping or after the said overlapping. Thus, the thermovolatile or thermosublimative coupler (a) is heat-transferred to the surface of the predetermined portion of the photosensitive material, and the light resolution of the diazonium salt (c) in the photosensitive material is caused to occur depending on the light transmission of the original. When the so exposed photosensitive material is developed by a method known per se, at the predetermined portion to which the coupler (a) has been heat-transferred, the diazonium salt (c) at the non-exposed area reacts selectively and preferentially with the coupler (a) to form a dyestuff (c) - (a) and at other portion the diazonium salt (c) at the non-exposed reacts with coupler (b) to form a dyestuff (c) - (b). Thus, there is obtained a multicolored reproductive copy in which the predetermined portion is colored in a hue different from that of the other portion.

The above-mentioned original for multicolor development may be prepared, for instance, by a method comprising applying a coating composition containing the above-mentioned thermovolatile or thermosublimative coupler (a) onto the back surface of a portion predetermined to have a different hue, of a transparent or semi-transparent original to be copied, or by a method comprising coating or impregnating a transparent or semi-transparent substrate with the said coating composition and combining the resulting sheet for heat-transferring the coupler, with the back surface of the specific portion of the original predetermined to have a different hue in a manner such that the layer for heat-transferring the coupler will confront the photosensitive material.

A coating composition for treating the back surface of an original and forming a layer for heat-transferring the coupler can be easily prepared by dispersing a coupler (a) into a liquid, semi-solid or solid dispersion medium.

Such treating agent will be now described by referring to some embodiments:

1. Ink-like composition for treating the back surface of an original:

|                      |            |
|----------------------|------------|
| Coupler (a)          | 5.0-25.0 % |
| Coloring material    | 0- 3.0 %   |
| Binder               | 0- 5.0 %   |
| Dispersion assistant | 0- 2.0 %   |
| Dispersion medium    | balance    |

As the dispersion medium there may be used water and organic solvents such as alcohol, toluene, xylene, esters and methyl ethyl ketone. It is possible to incorporate a coloring material so as to confirm the formation of a film of the treating agent, or to use a binder for the purpose of obtaining a good fixation of the coupler.

The composition of the above recipe is applied to the back surface of a portion predetermined to have a different hue by means of a brush, an installed felt pen, a ball pen, a coating roller, a sprayer or a printing machine.

2. Waxy composition for treating the back surface of an original:

|                   |             |
|-------------------|-------------|
| Coupler (a)       | 5.0-25.0 %  |
| Wax               | 85.0-15.0 % |
| Oil               | 10.0-40.0 % |
| Coloring material | 0-20.0 %    |

The composition of the above recipe is shaped to have a crayon stick-like form or a chalk-like form, and the back surface of a portion of an original predetermined to have a different hue is painted therewith. It is also possible to form a pressure-sensitive transfer sheet by melting the above composition or dissolving it in a suitable solvent and coating the melt or solution on a substrate such as paper and plastic film. The so formed pressure-sensitive transfer sheet is overlapped on the back surface of an original sheet, and then pressing is effected thereon by means of a typewriter or other writing means to form a heat-transferable layer on the back surface of an image predetermined to have a different hue.

3. Coupler-transferring sheet for treating the back surface of an original:

The ink-like composition for treating the back surface of an original, which was described in (1), or a composition obtained by incorporating a binder or an extender into such ink-like composition is coated on a transparent or semi-transparent sheet such as paper, plastic film or non-woven fabric. The so formed sheet for heat-transferring the coupler is cut into a desired size, if necessary, and then applied to the back surface of a portion of an original determined to have a different hue. It is possible to form a pressure-sensitive adhesive layer on the back surface of the coupler-transferring layer for preventing it from exfoliating from the original.

The so prepared original for multicolor development may be generally used 5 to 100 times repeatedly for the multi-color development, though the applicable frequency of the repeated use varies depending on the amount coated of coupler (a), the coating method, the heating method and the developing method. Of course, when the heat-transferability of coupler (a) in the layer for heat-transferring the coupler is lowered, it is sufficient to supply newly an additional layer for heat-transferring the coupler.

The exposure of the photosensitive material and the transfer of the thermovolatile or thermosublimative coupler (a) to the photosensitive surface may be effected coincidentally. For instance, in case a mercury lamp is used as light source for exposure, the heat transfer of the coupler (a) may be effected coincidentally with the exposure by the heat conveyed through a cylinder glass of the light source maintained at a relatively high temperature. Of course, the heat transfer of the coupler (a) may be also effected by the radiation heating of an image of the original. The heat transfer of the coupler (a) may be effectively performed by heating the layer for heat-transferring the coupler at a temperature above 50° C., preferably above 70° C., though a preferable heating temperature varies to some extent depending on the kind of the coupler (a) and the heating time. It is also possible to adopt a method comprising placing the above-mentioned original for multicolor development and the photosensitive material, passing the assembly through a heated roller or an infrared radiation zone to heat the layer for heat-transferring the coupler at the above-mentioned temperature and to effect the heat transfer of the coupler, and then passing the same through an exposure zone to effect the exposure of the photosensitive material.

It is also possible to adopt a method in which the exposure and heat transfer are conducted in an order reverse to that of the above method, namely a method comprising placing the original for multicolor development and the photosensitive material, passing the assembly through an exposure zone to effect the exposure of the photosensitive material and then passing the same through a heating zone to effect the heat transfer of the coupler (a).

In accordance with this invention, the photosensitive material which has been exposed to light and on a predetermined portion of which the coupler (a) has been heat-transferred, is developed by means known per se. The development may be conducted by either a dry method or a wet method.

In accordance with the dry process, the development may be performed sufficiently only by exposing the light-exposed photosensitive material to a mixture of ammonia and steam. In the case of the moist process the development can be accom-

plished by contacting the photosensitive material with an aqueous liquid developer containing an alkali.

In accordance with this invention there can be obtained multicolored reproductive copies in which the portions corresponding to predetermined portions of an original are colored selectively in different hues independently from other portions without any undesired mingling of colors. Further, multi-coloration can be accomplished by conducting the single-step development.

This invention will now be detailed by referring to accompanying drawings.

In the drawings,

FIGS. 1 and 2 are diagrams given to illustrate the multicolor reproduction process of this invention and

FIG. 3 is a CIE chromaticity diagram showing the results of Comparative Example in which the molar ratio of the coupler (b) to the diazonium salt (c) was varied, which Comparative Example will be detailed hereinbelow.

In the embodiment of this invention illustrated in FIG. 1, different thermovolatile or thermosublimative couplers 2' and 3' are coated on the back surfaces of images 2 and 3, respectively, of an original having images 1, 2 and 3. When the so formed original for multicolor development is placed on a photosensitive paper, and exposed to light emitted from a suitable light source, latent images 1'', 2'' and 3'' corresponding to images 1, 2 and 3 are formed on the photosensitive layer and couplers 2' and 3' are transferred on the upper surface of the photosensitive layer by the heat from the light source. When this photosensitive sheet is developed, the diazonium salt in latent images 2'' and 3'' of the photosensitive layer reacts selectively with transferred couplers 2' and 3', while the diazonium salt in latent image 1'' reacts with a coupler contained in the photosensitive layer. Thus, there is obtained a reproductive copy which has images 11, 12 and 13 colored in different hues.

FIG. 2 is a view illustrating an embodiment similar to the above embodiment shown in FIG. 1, except that a heat-transferable sheet containing coupler 2' and another heat-transferable sheet containing coupler 3' are applied to the back surfaces of images 2 and 3, respectively.

This invention will be now described by referring to examples.

#### EXAMPLES OF THE PREPARATION OF INK-LIKE AGENTS FOR TREATING THE BACK SURFACE OF AN ORIGINAL

##### Example A

An ink-like composition of the following recipe is prepared as a yellow color-forming agent for treating the back surface of an original:

|                     |         |
|---------------------|---------|
| Acetoacetic anilide | 20 g.   |
| Glycerin            | 15 g.   |
| Alkyd resin         | 5 g.    |
| Methanol            | 100 ml. |

The above composition is directly used as a material to be coated on the back surface of a portion of the original desired to be reproduced in yellow by means of a brush, a coating roller or a sprayer, or after it has been charged in a felt pen or a ball pen, it is used as a material for treating the back surface of a portion of the original desired to be reproduced in yellow.

##### Example B

An ink-like composition of the following recipe is prepared as a red color-forming agent for treating the back surface of an original:

|                                 |         |
|---------------------------------|---------|
| 1-Phenyl-3-methylpyrazolone (5) | 20 g.   |
| Styrene resin                   | 5 g.    |
| Glycerin                        | 15 g.   |
| Ethanol                         | 100 ml. |

The above composition is directly used as a material to be coated on the back surface of a portion of the original to be

reproduced in red by means of a brush, a coating roller or a sprayer, or after it has been charged in a felt pen or a ball pen, it is used as a material for treating the back surface of a portion of the original to be reproduced in red.

##### Example C

An ink-like composition of the following recipe is prepared as a brown color-forming agent for treating the back surface of an original:

|                     |         |
|---------------------|---------|
| Resorcinol          | 20 g.   |
| Vinyl acetate resin | 5 g.    |
| Glycerin            | 15 g.   |
| Methanol            | 100 ml. |

The above composition is directly used as a material to be coated on the back surface of a portion of the original desired to be reproduced in brown by means of a brush, a coating roller or a sprayer, or after it has been charged in a felt pen or a ball pen, it is used as a material for treating the back surface of a portion of the original desired to be reproduced in brown.

##### Example D

A blue-violet color-forming agent is prepared by using 2,3-dihydroxynaphthalene instead of acetoacetic anilide in the composition of Example A.

#### EXAMPLES OF THE PREPARATION OF WAXY AGENTS FOR TREATING THE BACK SURFACE OF AN ORIGINAL

##### Example E

A waxy composition to be used as a yellow color-forming agent for treating the back surface of an original is prepared by heat melting

|                     |        |
|---------------------|--------|
| Acetoacetic anilide | 30 g.  |
| Stearic acid        | 100 g. |
| Paraffin            | 50 g.  |
| Terra abla          | 50 g.  |
| Diatomaceous earth  | 20 g.  |

and solidifying the melt.

The above composition is molded into a crayon stick-like form and is used as a material to be coated on the back surface of a portion of the original desired to be reproduced into a different hue.

##### Example F

A waxy composition to be used as a yellowish brown color-forming agent for treating the back surface of an original is prepared by heat melting

|                             |        |
|-----------------------------|--------|
| Resorcinol monoglycol ether | 20 g.  |
| Paraffin                    | 50 g.  |
| Terra abla                  | 70 g.  |
| Haze wax                    | 20 g.  |
| Stearic acid                | 100 g. |
| Magnesium carbonate         | 20 g.  |

and solidifying the melt.

The so formed composition is molded into a crayon stick-like or chalk-like form and is used as a material for coating the back surface of a portion of an original desired to be reproduced in a different hue.

##### Example G

A waxy composition of the following recipe is prepared as a red color-forming agent for treating the back surface of an original:

|                                 |        |
|---------------------------------|--------|
| 1-Phenyl-3-methylpyrazolone (5) | 20 g.  |
| Stearic acid                    | 100 g. |
| Paraffin                        | 50 g.  |
| Diatomaceous earth              | 30 g.  |
| Haze wax                        | 20 g.  |

The above composition is molded into a crayon stick-like or chalk-like form and is used as a material for coating the back surface of a portion of the original desired to be reproduced in a different hue.

##### Example H

To the composition of Example G are added 100 g. of mineral oil, 50 g. oleic acid and 20 g. of Permanent Red, and the mixture is kneaded in a bowl mill to disperse additional components uniformly. Then, the kneaded mixture is coated on a substrate such as paper to obtain a pressure-sensitive copy sheet. The so formed copy sheet is overlapped on the back surface of an original and the pressing is effected thereon by means of a typewriter or other writing means. Thus, the sheet is used as a material for forming a layer of the waxy agent on the back surface of an image of the original to be reproduced in a different hue.

**EXAMPLES OF THE PREPARATION OF COUPLER-TRANSFERRING SHEETS FOR TREATING THE BACK SURFACE OF AN ORIGINAL**

**Example I**

A composition of the following recipe is prepared as a yellow color-forming agent for treating the back surface of an original:

|                          |        |
|--------------------------|--------|
| Acetoacetic acid aniline | 20 g.  |
| Triacetate resin         | 10 g.  |
| Methanol                 | 30 ml. |
| Acetone                  | 30 ml. |

The above composition is coated on a transparent or semi-transparent sheet such as polyester film by means of a rod coater and dried at a relatively low temperature (40° - 50° C.) to form a sheet for heat-transferring the coupler. After being cut into a desired size according to need, the sheet is used as a material to be applied to the back surface of a portion of an original desired to be reproduced in a different hue.

**Example J**

A composition to be used as a red color-forming agent for treating the back surface of an original is prepared by using 1-phenyl-3-methylpyrazolone (5) instead of acetoacetic acid aniline in Example I. From this composition there is formed a sheet for heat-transferring the coupler capable of forming a red color.

**Example K**

A composition to be used as a blue color-forming agent for treating the back surface of an original is prepared by using 2,3-dihydroxynaphthalene instead of acetoacetic acid aniline in Example I. From this composition there is formed a heat-transferable sheet capable of forming a blue color.

**Example L**

Multicolor-forming diazo-type photosensitive paper in use for dry development

A solution of the following recipe is prepared:

|                                                             |         |
|-------------------------------------------------------------|---------|
| 4-Diazo-N,N-dimethyl-aniline chloride 1/2 ZnCl <sub>2</sub> | 5 g.    |
| Diethylene glycol                                           | 60 g.   |
| Citric acid                                                 | 30 g.   |
| 2,3-Dihydroxynaphthalene-6-sulfonic acid                    | 15 g.   |
| Zinc chloride                                               | 50 g.   |
| Thiourea                                                    | 25 g.   |
| Patent Blue                                                 | 0.1 g.  |
| Water                                                       | balance |

The solution is coated on a base paper by a customary coating procedure such as using an air knife coater and dried to form a photosensitive sheet.

The sheet is overlapped on an original in which the back surface of a portion is treated with the treating material prepared in Example A and the back surface of another portion is treated with the treating material prepared in Example B. Then, the assembly is heated at 70° - 100° C. and exposed to light by means of a mercury lamp to form a latent image of the diazonium salt.

Next, the so treated sheet is subjected to development with gasified ammonia and steam. Thus, there is obtained a clear multicolor copy in which a portion corresponding to the portion treated with the material of Example A is colored in a yellow color, a portion corresponding to the portion treated with the material of Example B is colored in red and other portion corresponding to the untreated portion is colored in blue.

**Example 2**

When Example 1 is repeated by using 4-diazo-N-ethyl-N-hydroxyethyl-aniline chloride 1/2 ZnCl<sub>2</sub> instead of 4-diazo-N,N-dimethylaniline chloride 1/2 ZnCl<sub>2</sub>, there is obtained a multicolor reproductive copy similar to that of Example 1.

**Example 3**

Multicolor-forming photosensitive paper in use for dry development

A solution of the following recipe is prepared:

|                                                           |         |
|-----------------------------------------------------------|---------|
| 4-Diazo-N,N-diethylaniline chloride 1/2 ZnCl <sub>2</sub> | 15 g.   |
| Glycerine                                                 | 50 g.   |
| Citric acid                                               | 40 g.   |
| 2-naphthol-3,6-disulfonic acid                            | 6 g.    |
| Zinc chloride                                             | 25 g.   |
| Thiourea                                                  | 25 g.   |
| Patent Blue                                               | 0.1 g.  |
| Water                                                     | balance |

Total 1 liter

By a customary coating method such as using an air knife coater, a photosensitive paper is prepared from the above solution. The photosensitive paper is placed on an original in which a portion of the back surface is treated with the waxy composition prepared in Example E and another portion of the back surface is treated with the composition prepared in Example G. The assembly is exposed to light and heated by means of a mercury lamp. Then, the so treated sheet is subjected to development with gasified ammonia and steam. Thus, there is obtained a clear three-color reproductive copy in which a portion corresponding to the portion of the original treated with the composition of Example E is colored in yellow, a portion corresponding to the portion treated with the composition of Example G is colored in red, and other portion corresponding to the untreated portion of the original is colored in bluish violet.

**Example 4**

Multicolor-forming photosensitive paper in use for dry development

A solution of the following recipe is prepared:

|                                                            |         |
|------------------------------------------------------------|---------|
| 4-Diazo-N,N-dimethylaniline chloride 1/2 ZnCl <sub>2</sub> | 20 g.   |
| Diethylene glycol                                          | 50 g.   |
| Citric acid                                                | 50 g.   |
| 2,7-Dihydroxynaphthalene-3,6-disulfonic acid sodium salt   | 8 g.    |
| Resorcinol monoethyl ether                                 | 2 g.    |
| Zinc chloride                                              | 10 g.   |
| Thiourea                                                   | 50 g.   |
| 1,3,6-Naphthalene-trisulfonic acid sodium salt             | 20 g.   |
| Patent Blue                                                | 0.1 g.  |
| Water                                                      | balance |

Total 1 liter

In the same manner as in Example 1, a photosensitive paper is prepared from the above solution by coating and drying. The photosensitive paper is placed on an original, a portion of the back surface of which is treated with the coupler-heat-transferring sheet prepared in Example J and another portion of the back surface of which is treated with the treating agent

obtained in Example K. Then the assembly is heated and printed by means of a mercury lamp, followed by development with gaseous ammonia and steam. Thus there is obtained a clear three-color reproductive copy in which a portion corresponding to the portion treated with the treating agent of Example J is colored in red, another portion corresponding to the portion corresponding to the portion treated with the treating agent of Example K is colored in blue and the remaining portion corresponding to the untreated portion is colored in black.

Example 5

Multicolor-forming photosensitive paper for dry development

A solution of the following recipe is prepared:

|                                        |         |         |
|----------------------------------------|---------|---------|
| 4-Diazo-N,N-dimethylaniline chloride   | 20      | g.      |
| Ethylene glycol                        | 50      | g.      |
| 2,4,2',4'-Tetrahydroxydiphenyl sulfide | 11      | g.      |
| Thiourea                               | 25      | g.      |
| Zinc chloride                          | 50      | g.      |
| Patent Blue                            | 0.1     | g.      |
| Water                                  | balance |         |
| <b>Total</b>                           |         | 1 liter |

The above solution is coated on a semi-transparent paper such as tracing paper and dried to form a photosensitive paper. The photosensitive paper is placed on an original, a portion of the back surface of which is treated with the ink-like composition prepared in Example B and another portion of the back surface of which is treated with the composition obtained in Example D. Then the assembly is heated and printed by means of a mercury lamp, followed by development with gaseous ammonia and steam. Thus there is obtained a clear three-color reproductive copy usable as the intermediate in which a portion corresponding to the portion of the original treated with the composition of Example B is colored in red, another portion corresponding to the portion treated with the composition of Example D is colored in blue and other portion corresponding to the untreated portion of the original is colored in yellowish brown.

Example 6

Multi-color-forming photosensitive paper for dry development

A solution of the following recipe is prepared:

|                                                                     |         |         |
|---------------------------------------------------------------------|---------|---------|
| 4-Diazo-N-ethyl-N-hydroxyethylaniline chloride 1/2ZnCl <sub>2</sub> | 20      | g.      |
| Diethylene glycol                                                   | 75      | g.      |
| Tartaric acid                                                       | 40      | g.      |
| α-resorcylic acid amine                                             | 8       | g.      |
| Zinc chloride                                                       | 50      | g.      |
| Thiourea                                                            | 25      | g.      |
| Patent Blue                                                         | 0.1     | g.      |
| Water                                                               | balance |         |
| <b>Total</b>                                                        |         | 1 liter |

By a customary coating method such as using an air knife coater, the above solution is applied to a substrate of a photosensitive paper and dried. The so formed photosensitive paper is placed on an original, a portion of the back surface of which is treated with a coupler-heat-transferring sheet prepared in Example K, and the assembly is heated and printed by means of a mercury lamp, followed by development with gaseous ammonia and steam. Thus there is obtained a clear two-color reproductive copy without any substantial mingling of colors, in which a portion corresponding to the portion of the original treated with the sheet obtained in Example K is colored in blue and the remaining portion cor-

65  
70

responding to the untreated portion of the original is colored in red.

Example 7

Multicolor-forming photosensitive paper for dry development

A solution of the following recipe is prepared:

|    |                                          |         |         |
|----|------------------------------------------|---------|---------|
| 10 | 4-Diazo-N,N-diethylaniline               |         |         |
|    | .1/2ZnCl <sub>2</sub>                    | 20      | g.      |
|    | Ethylene glycol                          | 50      | g.      |
|    | Citric acid                              | 20      | g.      |
|    | Bis-(5-hydroxy-7-sulfonaphthyl(2))-amine | 14      | g.      |
|    | Zinc chloride                            | 30      | g.      |
|    | Thiourea                                 | 25      | g.      |
|    | Hydrochloric acid (36%)                  | 10      | ml.     |
|    | Patent Blue                              | 0.1     | g.      |
|    | Water                                    | balance |         |
|    | <b>Total</b>                             |         | 1 liter |

20 The above solution is applied to a photosensitive paper substrate by a customary coating method such as using an air knife coater, and the resulting photosensitive paper is placed on an original, a portion of the back surface of which is treated with the ink-like composition obtained in Example C. The assembly is heated and printed by means of a mercury lamp, followed by development with gaseous ammonia and steam. Thus there is obtained a clear two-color reproductive copy in which a portion corresponding to the treated portion of the original is colored in brown and other remaining portion corresponding to the untreated portion of the original is colored in dark blue.

Example 8

Multicolor-forming sensitive paper in use for either dry or wet development

A solution of the following recipe is prepared:

|    |                                                              |         |         |
|----|--------------------------------------------------------------|---------|---------|
| 40 | 4-Diazo-2,5-dibutoxy-N-phenylmorpholine 1/2ZnCl <sub>2</sub> | 15      | g.      |
|    | Citric acid                                                  | 30      | g.      |
|    | Diethylene glycol                                            | 40      | g.      |
|    | β-Hydroxynaphthonic acid aminoethyl amine (hydrochloride)    | 7       | g.      |
|    | Thiourea                                                     | 40      | g.      |
|    | Zinc chloride                                                | 30      | g.      |
|    | Patent Blue                                                  | 0.1     | g.      |
|    | Water                                                        | balance |         |
|    | <b>Total</b>                                                 |         | 1 liter |

50 From the above solution, a photosensitive paper is prepared by conducting the coating and drying in the same manner as in Example 1. The so formed photosensitive paper is piled on an original, a portion of the back surface of which is treated with the ink-like composition prepared in Example A and another portion of the back surface of which is treated with the treating material prepared in Example C. Then the assembly is heated and printed by means of a mercury lamp, followed by development with gaseous ammonia and steam or with an alkaline liquid developer of the following recipe:

|    |                       |         |         |
|----|-----------------------|---------|---------|
| 65 | Potassium carbonate   | 30      | g.      |
|    | Sodium thiosulfate    | 40      | g.      |
|    | Sodium bicarbonate    | 30      | g.      |
|    | Potassium tetraborate | 5       | g.      |
|    | Water                 | balance |         |
|    | <b>Total</b>          |         | 1 liter |

70 Thus there is obtained a clear three-color reproductive copy without any substantial mingling of colors, in which a portion corresponding to the portion of the original treated with the

composition of Example A is colored in yellow, a portion corresponding to the portion of the original treated with the composition of Example C is colored in brown and the remaining portion corresponding to the untreated portion of the original is colored in blue.

#### Example 9

##### Multicolor-forming film

A solution of the following recipe is prepared:

|                                                                |     |     |
|----------------------------------------------------------------|-----|-----|
| 4-diazo-2,5-dibutoxy-N-phenyl morpholine-1/2 ZnCl <sub>2</sub> | 15  | g.  |
| Citric acid                                                    | 8   | g.  |
| β-Hydroxynaphthoic acid                                        |     |     |
| ethanol amine                                                  | 7   | g.  |
| Triacetate resin                                               | 15  | g.  |
| Oil Blue                                                       | 0.2 | g.  |
| Acetone                                                        | 600 | ml. |
| Methanol                                                       | 400 | ml. |

The solution is coated on a polyester film by a rod coater and dried at a relatively low temperature (40° - 50°C.) by warm air to form a photosensitive film. The film is placed on an original in which a part of the back surface of an original image is treated with the ink-like agent prepared in Example A and another part of the back surface of the original image is treated with the treating agent prepared in Example B. The assembly is exposed to light by a mercury lamp and heated and printed. The photosensitive film containing a latent image of the diazonium salt is developed with gasified ammonium and steam. Thus, there is obtained a clear three-color reproductive copy without any substantial mingling of colors, in which a portion corresponding to the part treated with the treating material of Example A is colored in yellow, a portion corresponding to the part treated with the treating material of Example B is colored in red, and other portion corresponding to the untreated part of the original is colored in blue.

#### Comparative Example

This example is given to illustrate the relation between the amount of the coupler (b) (having a lower coupling rate than the thermovolatile or thermosublimative coupler (a)) and the effect of preventing the mingling of colors.

#### Experimental Procedures;

Each of sample solutions having the following composition and containing MA salt and DS acid at a molar ratio, indicated

45

TABLE 1

| Sample No. | Molar Ratio |         |
|------------|-------------|---------|
|            | MA salt     | DS acid |
| 5          |             |         |
| 10         | 1           | 0.25    |
| 10         | 1           | 0.5     |
| 10         | 1           | 0.75    |
| 10         | 1           | 1       |
| 10         | 1           | 1.5     |
| 10         | 1           | 2       |
| 10         | 1           | 2.5     |
| 10         | 1           | 3       |
| 10         | 1           | 3.5     |
| 15         | 1           | 4       |

Each of the so formed photosensitive papers is placed on a non-transparent original, a portion of the back surface of which is treated with a treating composition (20 percent solution of resorcinol in ethanol), and the assembly is heat-treated at 70° C. for 4 seconds and subjected to development with gaseous ammonia and steam. Then the degree of distinction in developed colors is examined with respect to each sample. The examination is conducted in accordance with the method of JIS-Z-8722 using a color-difference meter (CS-4A) of Nippon Denshoku Kabushiki Kaisha in the following manner:

The color tones of the portion corresponding to the treated portion of the original and the portion corresponding to the untreated portion of the original are determined by measuring tristimulus values X, Y and Z according to colorimetric system CIE. Then the values of x and y are calculated by the following equations:

$$x = X/X+Y+Z \quad y = Y/X+Y+Z$$

Based on these values the dominant wavelength ( $\lambda$  max) and excitation purity (Pe) are determined from the CIE standard chromaticity diagram, and the effect of preventing the mingling of colors is evaluated from the deviation of the dominant wavelength and the change in excitation purity.

40 In order to determine the color difference ( $\Delta E$ ) between the two colored hues, values of L, a and b defined in UCS colorimetric system are measured, and the value of  $\Delta E$  is calculated from the following equation:

$$\Delta E = \sqrt{(\Delta L)^2 + (\Delta a)^2 + (\Delta b)^2}$$

Results are shown in Table 2.

TABLE 2

| Sample No. | Portion corresponding to untreated portion of original |                                 | Portion corresponding to treated portion of original |                                                | Color difference between portions corresponding to treated and untreated portions of original ( $\Delta E$ ) |
|------------|--------------------------------------------------------|---------------------------------|------------------------------------------------------|------------------------------------------------|--------------------------------------------------------------------------------------------------------------|
|            | Dominant wavelength ( $\lambda$ max.), m $\mu$         | Excitation purity (Pe), percent | Sample No.                                           | Dominant wavelength ( $\lambda$ max.), m $\mu$ |                                                                                                              |
| 1          | 458                                                    | 26                              | 1'                                                   | 585                                            | 42                                                                                                           |
| 2          | 450                                                    | 33.5                            | 2'                                                   | 586.5                                          | 38                                                                                                           |
| 3          | 400                                                    | 37                              | 3'                                                   | 588.5                                          | 34.5                                                                                                         |
| 4          | -565.3                                                 | 41.5                            | 4'                                                   | 589                                            | 26                                                                                                           |
| 5          | -564.5                                                 | 46                              | 5'                                                   | 594                                            | 21                                                                                                           |
| 6          | -563.3                                                 | 48                              | 6'                                                   | 611                                            | 13.6                                                                                                         |
| 7          | -564.3                                                 | 51                              | 7'                                                   | -493.5                                         | 12                                                                                                           |
| 8          | -563.5                                                 | 52                              | 8'                                                   | -495.5                                         | 13.8                                                                                                         |
| 9          | -564.5                                                 | 52.5                            | 9'                                                   | -503                                           | 16                                                                                                           |
| 10         | -564                                                   | 56                              | 10'                                                  | -527                                           | 22.5                                                                                                         |

in Table 1 is coated by hand on a photosensitive paper substrate:

65

#### NOTES

1. The value of dominant wavelength expressed in minus is the value of complementary dominant wavelength.

2. The unit of  $\Delta E$  is the NBS unit.

70 The above results are plotted on the CIE chromaticity diagram and shown in FIG. 3.

From the above results the following matters can be seen:

With reference to the color tone in the portion corresponding to the treated portion of the original, if the coupler (b) (DS acid) is used in an amount such that its molar ratio to the diazonium (c) (MA salt) is 1 or more (samples 4 - 10), the

|                                                                      |          |
|----------------------------------------------------------------------|----------|
| 4-Diazo-N,N-dimethylaniline chloride-1/2 ZnCl <sub>2</sub> (MA salt) | variable |
| Diethylene glycol                                                    | 60 g.    |
| Citric acid                                                          | 40 g.    |
| 2,3-Dihydroxynaphthalene-6-sulfonic acid (DS acid)                   | variable |
| Zinc chloride                                                        | 50 g.    |
| Thiourea                                                             | 25 g.    |

dominant wavelength deviates toward the long wavelength area, and at the molar ratio of 2.5 (sample 7) the dominant wavelength comes to be in the range of the complementary dominant wavelength, with the result that the color tone becomes close to the color tone of the portion corresponding to the untreated portion of the original, namely the color tone becomes closer to bluish violet. With reference to excitation purity ( $P_e$ ), when the amount used of the coupler (*b*) (DS acid) is increased and the above-mentioned molar ratio is 1 or more (samples 4 - 10), the distinctness of color is lowered with the decrease of the value of excitation purity to less than 25 percent, with the result that darkening of color is caused to appear and the color distinction becomes bad.

On the other hand, in case the above-mentioned molar ratio is less than 1, namely in case the coupler (*b*) is used in an amount such as will result in the dominant wavelength of 585 - 589  $m\mu$  and excitation purity of more than 25 percent, the color distinction is excellent and a suitable photosensitive paper is obtainable.

With reference to the portion corresponding to the untreated portion of the original, the increase of the amount used of the coupler (*b*) (DS acid) results in increase of excitation purity and color distinctness. However, in each sample the excitation purity is above 25 percent and there is no great change in the dominant wavelength except sample 1. Accordingly, from the viewpoint of definite color distinction, samples 1 - 4 (where the above-mentioned molar ratio is in the range of 0.25 - 1) are suitable as photosensitive paper. The values of the color difference ( $\Delta E$ ) between the two colors are considerably different from the values actually found. This is due to the fact that while the value of  $\Delta E$  conforms to the actually found value at the center of the chromatocity diagram, in the marginal portion where the color is denser the calculated value of  $\Delta E$  is inaccurate. Thus these values of the color difference  $\Delta E$  are given only for reference.

What we claim is:

1. A process for the diazo-type multicolor reproduction which comprises conducting the steps of (A) exposing imagewise to actinic light a diazo-type photosensitive material

- having a photosensitive layer containing at least one photosensitive diazonium salt (*c*) and an azo coupler (*b*) having a substantially lower rate of coupling with the diazonium salt (*c*) than that of resorcinol, said azo-coupler being present in the 5 photosensitive layer in an amount of from 0.1 to 1 mole per mole of said diazonium salt (*c*), and (B) heating at a predetermined portion a layer of at least one thermovolatile or thermosublimative azo coupler (*a*) which is disposed in face-to-face contact with said photosensitive material to produce an 10 azo dye image in the area of the diazotype material contiguous with the heated area of the layer containing azo coupler (*a*), said steps being performed coincidentally or in the order of (A) to (B) or (B) to (A), and then developing the exposed 15 photosensitive material to produce an azo dye image in the unexposed area of said diazo-type material which is a different hue or color from the azo dye image formed by heating.
2. The process as described in claim 1 wherein the exposed photosensitive material is developed with ammonia and steam or with an aqueous liquid developer containing an alkali.
- 20 3. The process as described in claim 1 wherein a transparent or semi-transparent layer, containing at least one thermovolatile or thermosublimative azo coupler (*a*), is applied to the back surface of a predetermined portion of a transparent or semi-transparent original and then placed on the photosensitive diazo-type material such that the photosensitive layer will be in face-to-face contact with the layer containing azo coupler (*a*), and both the light exposure and heat transfer of azo coupler (*a*) are performed when the composite structure is in the above described relationship.
- 25 4. The process as described in claim 1 wherein a dyestuff formed from the coupler (*b*) and the diazonium salt (*c*) exhibits a hue different from a hue of a dyestuff formed from the thermovolatile or thermosublimative coupler (*a*) and the diazonium salt (*c*).
- 30 5. The process as described in claim 1 wherein in the photosensitive layer of the photosensitive material the coupler (*b*) is present in an amount of 0.2 - 0.9 mole per mole of the diazonium salt (*c*).

\* \* \* \* \*

40

45

50

55

60

65

70

75